

July 27, 1965

A. T. BALEVSKY ET AL

3,196,501

APPARATUS AND METHOD FOR METAL CASTING

Filed Feb. 13, 1962



FIG. 1



FIG. 2a



FIG. 3



FIG. 2b

INVENTORS.  
ANGEL TONSCHEV BALEVSKY  
IVAN DIMOV NIKOLOV  
BY

*M. G. Lew & Toren*  
ATTORNEYS.

## 1

3,196,501

APPARATUS AND METHOD FOR METAL  
CASTINGAngel T. Balevsky and Ivan D. Nikolov, Sofia, Bulgaria,  
assignors to Bulgarska Akademia Na Naukite, Sofia,  
Bulgaria

Filed Feb. 13, 1962, Ser. No. 173,052

10 Claims. (Cl. 22—68)

This invention relates in general to metal casting apparatus and to a method of casting; and, in particular, to an improved apparatus and method for casting materials using counter-pressure.

The present invention refers particularly to pressure casting. At the present time it is usual when casting under pressure to direct the molten metal into a pressmold or pressure mold in the form of a jet under pressure exerted by a pressure producing means such as a movable piston or a compressed air reserve tank. A disadvantage of such method is that intense whirling of the molten metal with the air or gases in the pressmold takes place and this results in the entrapment of the air or gases in the molten mass making the resultant cast pieces porous. With such prior art methods, the pressmold is subjected to atmospheric pressure and the casting can be subjected to high pressure only after the mold is filled up at which time the air in the mold already mixes with the molten metal and the solidifying of the metal in some portions of the casting has already begun. This results in disadvantageous blowholes in the casting due to the bubbles of air or gases which become entrapped in the casting. When attempts are made to exert extremely high pressures on the casting in order to reduce the size of such bubbles and to obtain a more precise casting, the apparatus becomes unusually expensive or the dimensions and weight limits of the casting are unduly restricted.

In accordance with the present invention the casting is formed by subjecting the mold to a pressure which advantageously may be regulated to desired amounts above atmosphere and by imposing a larger pressure on the molten metal which is injected into the mold. With such a method and apparatus to effect the same, the disadvantages mentioned above are eliminated. The improved method and apparatus are effected by controlling the pressure within the mold as well as the pressure of the molten metal being injected thereinto. In this manner it is possible to regulate the speed at which the molten metal rises in the pressmold in a way so that neither breaking of the free surface nor mixing of the molten metal with air or gases results. In addition, in accordance with this method it is also possible to maintain the pressmold and the molten metal therein under the continuous action of a preliminary predetermined pressure insuring in this manner the production of an exact impression.

In accordance with one embodiment of the apparatus a pressmold is arranged between a pressure compensating chamber and molten metal feeding reservoir and a compressed air reservoir is employed to selectively pressurize the compensation chamber and the feeding reservoir which communicates at opposite sides with the pressmold for the purpose of regulating the pressure acting on each side of the mold.

In still another embodiment of the invention there is provided a rotatable apparatus which includes a pressmold and a molten metal reservoir communicating with the mold. The mold in turn is connected at its opposite end with a pressurized fluid source and the pressurized fluid source is also communicated with the molten metal reservoir. When the apparatus is rotated, the molten metal reservoir is disposed above the mold so that the molten metal flows down under the gravity head of the

## 2

height of molten metal in the reservoir above the mold. Additional pressure regulation is achieved by the compressed air reservoir to regulate the pressure acting downwardly on the molten liquid to force it into the mold and to regulate the pressure acting on the top of the mold upon the surface of the liquid as it is being moved upwardly into the mold.

In still another embodiment of the invention there is provided a reservoir of molten liquid which communicates directly with the pressure mold at the lower end thereof and valve means for regulating the pressure at the upper end of the mold. A piston is arranged to act upon the liquid in the molten liquid reservoir to force it into the pressure mold against the pressure which acts on the upper end thereof.

Accordingly, it is an object of this invention to provide an improved method for casting metals under pressure.

A further object of the invention is to provide an apparatus for casting metals under pressure.

A further object of the invention is to provide a method of casting metals under pressure which includes pressurizing one side of a mold and directing molten metal into the opposite side of the mold by a greater pressure regulated to permit uniform rising in the mold without turbulence or entrainment of fluid in the molten metal.

A further object of the invention is to provide an improved device for casting metals under pressure which includes a pressure mold which is connected to a reservoir for feeding molten liquids thereto at one end and is subjected to a pressure above atmospheric at its opposite end and means for regulating the pressure to permit the rising of the metal into the mold while maintaining the metal at a pressure above atmosphere.

A further object of the invention is to provide a method and apparatus for casting under pressure which is simple in concept, economical to carry out and provides a casting of improved characteristics.

The various features of novelty which characterize the invention are pointed out with particularity in the claims annexed to and forming a part of this specification. For a better understanding of the invention, its operating advantages and specific objects attained by its use, reference should be had to the accompanying drawings and descriptive matter in which there are illustrated and described preferred embodiments of the invention.

In the drawings:

FIG. 1 is a diagrammatic illustration of an apparatus for casting metals under pressure constructed in accordance with the invention;

FIG. 2a is a diagrammatic illustration of another embodiment of the apparatus for casting metals under pressure;

FIG. 2b is a diagrammatic illustration of the apparatus indicated in FIG. 2a but with the parts oriented in an operating position; and

FIG. 3 is a diagrammatic illustration of still another embodiment of the invention.

Referring to the drawings in particular, as indicated in FIG. 1 the invention includes a pressure mold or pressmold 3 which is provided with a gas permeable outlet 4 at one side and which is provided with a connection to a runner or filler tube 2 at the opposite side. Molten metal is maintained in a feeding reservoir 1 in direct communication with the lower end of the runner tube 2. The gas permeable outlet 4 is covered by a housing to form a pressure compensating chamber 5.

In accordance with the invention, pressure acting on the mold designated  $P_2$  is regulated to an amount advantageously above atmosphere by directing compressed fluid from a compressed fluid reservoir R through conduits 10 and 12 to the pressure compensating chamber 5.

A further control on this pressure is obtained by regulating a discharge valve *c* in a conduit 14.

Initially the pressure  $P_2$  acting on the press mold 3 and the pressure  $P_1$  in the feed reservoir 1 are equal. For example, this pressure can be 1, 5, 10, 20 etc. atmospheres, according to the requirements of the particular case. This pressure may be produced, for example, by introduction of a compressed gas, such as air, from the fluid reservoir R.

Such materials as aluminum alloys, zinc alloys, iron, or the like, may be cast in the apparatus indicated in the drawings. The temperatures and pressures required will be a function of the type of metal or alloy which is to be cast, the form and size of the press mold 3, and the rate of cooling. Those skilled in the art will readily be able to determine the particular temperatures and pressures required.

When it is desired to direct the metal from the feeding reservoir 1 into the pressure mold 3, compressed fluid is directed from the conduit 10 through a conduit 16 by opening valves *d* and *b* in conduits 10 and 16, respectively. Valve *a* in conduit 12 and valve *c* in conduit 14 are regulated along with valves *d* and *b* to insure that the pressure  $P_2$  is above atmosphere, but that the pressure  $P_1$  acting downwardly on the molten metal to cause it to feed through the runner tube 2 is greater than the pressure  $P_2$  acting on the top surface of the metal as it rises in the pressure mold 3. Thus, it is possible with the arrangement outlined to accurately control the speed at which the molten metal will enter into the pressure mold 3 as determined by the differential in pressure between  $P_1$  and  $P_2$ . It is possible in accordance with the invention to choose the pressure differential so that the molten metal remains unbroken as it feeds into the mold 3 and insure that air and other gases existing in the pressure mold will not form as bubbles within the metal which is being cast. By maintaining the metal which is being cast under the influence of the pressure  $P_2$  during the casting operation, it is further insured that the exact reproduction of the shape of the mold will be produced in the casting.

In FIG. 2, a modified apparatus is indicated which comprises a rotatable structure including a spherical molten metal reservoir 20, a pressure mold 22 which communicates with the molten metal reservoir through an opening 24, and a fluid pressure reservoir 26 which communicates with the molten metal reservoir through conduits 28 and 30 and with the pressure mold 22 through the conduits 28 and 32. In the position indicated in FIG. 2a, the apparatus is shown prior to the directing of the molten metal into the pressure mold 22.

In FIG. 2b the apparatus is shown rotated to a position in which the molten metal reservoir 20 is disposed above the pressmold 22 so that there will be a tendency for the weight of the molten metal to cause flow downwardly through the opening 24 into the pressmold 22. The pressmold 22 includes an elongated narrow passage 22a extending downwardly from the opening 24 and a widened portion 22b which communicates through a gas permeable outlet 34 to conduit 32. The pressure  $P_a$  in the molten metal reservoir 20 is regulated by directing fluid from the fluid pressure source 26 through conduit 28 and valve *a* to the conduit 30 leading to the reservoir 20. In addition, the pressure acting at  $P_b$  in the chamber 22b of the pressure mold 22 is controlled by directing pressure from the fluid pressure source 26 through conduit 28 and conduit 32 as regulated by valves *a*, *b* and *c*.

In the embodiment indicated in FIG. 3, a pressmold 36 is provided with an opening 38 at its lower end which communicates through a tube 40 with a reservoir 42 of molten metal. The molten metal is directed into the lower end of the pressure mold 36 by means of a piston 44 by the application of a downward force  $P$  indicated by the arrow. The pressure at the top of the mold is controlled by a valve 46 in a conduit 48 which communicates through a fluid permeable outlet 50 to the top of the mold

36. In the embodiment, the pressure mold 36 can be gradually filled with molten metal under the control of pressure created by the force of the piston 44 and the pressure which exists at the top of the mold 36.

While a specific embodiment of the invention has been shown and described in detail to illustrate the application of the inventive principles, it will be understood that the invention may be embodied otherwise without departing from such principles.

What is claimed is:

1. A pressure casting device comprising, in combination, a mold, a liquefied material reservoir connected to said mold, means for applying the same super atmospheric pressure to both said mold and said liquefied material reservoir, means for establishing a pressure differential between said reservoir and said mold, while maintaining the pressures at said reservoir and said mold at super atmospheric values with the pressure at the mold being less than the pressure at the liquefied material reservoir, to cause the liquefied material to flow from the reservoir to mold to fill the mold gradually, and means for maintaining said pressure differential constant during the entire process of filling the mold.

2. A pressure casting device, as claimed in claim 1, wherein said mold has an air permeable outlet on one side, said means for applying super atmospheric pressure and for maintaining a constant pressure differential comprising a fluid pressure reservoir connected to said air permeable outlet and to said liquid material reservoir, and valve means to regulate the pressure acting on said outlet and on said liquid material reservoir.

3. A device according to claim 2, including a pressure compensating chamber surrounding said outlet, said pressure compensating chamber being connected to said fluid pressure reservoir.

4. A pressure casting device according to claim 1, wherein one side of said mold is provided with a fluid permeable outlet.

5. A pressure casting device according to claim 1, including a piston acting on said liquefied material to pressurize the material to cause it to flow into said mold.

6. In a method of casting liquefied material by feeding the liquefied material from a reservoir thereof to a mold: the improvement comprising, in advance of feeding metal to the mold, subjecting the reservoir and the mold to the same super atmospheric pressure; then establishing a pressure differential between the reservoir and the mold, while maintaining the pressures in both the reservoir and the mold at a super atmospheric value with the pressure in the mold being less than that in the reservoir, whereby to cause the liquefied material to flow from the reservoir into the mold and gradually to fill the mold; and maintaining such pressure differential constant during the entire mold filling process.

7. In a method of casting liquefied material as claimed in claim 6, the improvement comprising controlling the speed at which the liquefied material enters the mold by adjusting the pressure differential between the reservoir and the mold.

8. In a method of casting liquefied material, as claimed in claim 6, the improvement wherein the pressure in the reservoir is produced by means of a direct acting piston, while the pressure in the mold is produced by a compressed gas.

9. A pressure casting device comprising, in combination, a mold, a liquefied material reservoir connected to said mold, means for applying the same super atmospheric pressure to both said mold and said liquefied material reservoir, means for establishing a pressure differential between said reservoir and said mold while maintaining the pressures at said reservoir and said mold at super atmospheric values with the pressure at the mold being less than the pressure at the liquefied material reservoir, to cause the liquefied material to flow from the

reservoir to mold to fill the mold gradually, and means for maintaining said pressure differential constant during the entire process of filling the mold, said liquefied material being maintained in a closed vessel communicating with said mold, said vessel and said mold being rotatable to position said vessel above said mold to permit the flow of the material into the mold under the influence of the weight of the material above said mold.

10. A pressure casting device comprising, in combination, a mold, a liquefied material reservoir connected to said mold, means for applying the same superatmospheric pressure to both said mold and said liquefied material reservoir, means for establishing a pressure differential between said reservoir and said mold, while maintaining the pressure at said reservoir and said mold at superatmospheric values with the pressure at the mold being less than the pressure at the liquefied material reservoir, to cause the liquefied material to flow from the liquefied material reservoir to mold to fill the mold gradually, and means for maintaining said pressure differential constant

during the entire process of filling the mold, including a reservoir of fluid under pressure connected to one side of said mold and to said liquefied material reservoir.

References Cited by the Examiner

UNITED STATES PATENTS

|           |      |            |       |        |
|-----------|------|------------|-------|--------|
| 2,210,544 | 8/40 | Galloway   | ----- | 22—69  |
| 2,310,766 | 2/43 | Dornauf    | ----- | 22—209 |
| 2,821,757 | 2/58 | Wood       | ----- | 22—69  |
| 2,994,115 | 8/61 | Schuchardt | ----- | 22—68  |
| 2,997,756 | 8/61 | Strom      | ----- | 22—69  |
| 3,032,841 | 5/62 | Sylvester  | ----- | 22—69  |

FOREIGN PATENTS

|    |        |      |                |
|----|--------|------|----------------|
| 15 | 11,423 | 7/09 | Great Britain. |
|----|--------|------|----------------|

J. SPENCER OVERHOLSER, *Primary Examiner.*

WINSTON A. DOUGLAS, MARCUS U. LYONS,  
20 MICHAEL V. BRINDISI, *Examiners.*